

## UNITED STATES PATENT OFFICE

1,971,149

## PURIFICATION OF MOLTEN METAL

William F. Zimmerli, Niagara Falls, N. Y., assignor to E. I. du Pont de Nemours & Company, Incorporated, Wilmington, Del., a corporation of Delaware

No Drawing. Application September 12, 1932,  
Serial No. 632,794

3 Claims. (Cl. 75—62)

This invention relates to the purification of metals or alloys, particularly to the treatment of molten iron, steel, copper, brass or the like with sodium cyanide or other metal cyanides or 5 equivalent cyanogen derivatives.

In the manufacture and purification of such metals and alloys, considerable difficulty is experienced, due to the partial oxidation of the metal, resulting in the occlusion of oxides which detract 10 from the desirable physical properties of the product. This difficulty is partially corrected by the addition of deoxidizing agents which reduce these oxides. The present treating materials do not give entirely satisfactory results in many cases 15 because they either form oxides of other metals in the melts, or because an excess of the treating material itself adversely affects the quality of the product. Thus, aluminum has been found to be an efficient medium in reducing iron oxide in 20 molten steel, but the aluminum oxide itself is largely occluded in the final product. While the steel is improved, it would be more desirable to reduce the iron oxide by some other method which would not leave an undesirable residue. In the 25 case of copper it has been found that calcium is an effective deoxidizing material, but an excess of calcium remaining in the copper reduces the electrical conductivity. In the treatment of brass, bronze, and copper the element, phosphorus, is commonly used in the form of its copper 30 alloy, but in many cases an excess of this in the alloy is objectionable.

The object of this invention is to provide a satisfactory treating means and material for such 35 molten metals which will not leave these objectionable residues in the product to detract from desirable physical properties.

I have found that these results can be secured by the treatment of the molten metal with a cyanogen compound, and more specifically a cyanogen salt such as a metal cyanide, cyanate, thiocyanate, or other cyanogen derivatives. Such metal cyanides as sodium cyanide, copper cyanide or the like can be used. Thus, copper cyanide 45 can be used for the treatment of copper and the final reaction product remaining in the metal would be pure copper.

Alkali metal cyanides, such as sodium cyanides, are effective to product these results. The alkali 50 metal cyanides do not decompose violently when heated to high temperatures in the absence of oxygen or compounds containing oxygen; however, they are very active with metallic oxides, reducing these to metals. In the reducing reaction, cyanides are oxidized to cyanates, and cya-

nates eventually transform to carbonates. At the temperature of molten steel, for example, with very small amounts of reducible oxide, the products formed would probably vary considerably; however, iron oxide would be reduced, and the 60 cyanide would leave an alkali compound which would be easily fusible so that it would come out of the molten metal as a slag. Other impurities, such as occluded oxide silicon, manganese, and other metals taken up from the linings of the furnaces, slags, etc., or produced by the additions of the elements to effect deoxidation or desulphurization, would either be reduced or converted to fusible slags easily removable from the metals.

As noted above, metal cyanides of the constituents of the final product would be preferable in cases where small amounts of foreign elements would give lower quality products. Thus, as noted above, copper can be deoxidized with pure copper cyanide, so that the final reaction product remaining in the metal is pure copper. If the copper were first deoxidized with calcium, an excess of this can be removed by adding copper cyanide.

After treatment of the molten metal with 80 cyanide carrying material, it may be advantageous to treat the metal with a degasifying agent. For this purpose any of the common degasifiers suited for this particular metal may be used.

I have in this manner treated molten steel 85 with sodium cyanide, and molten copper with sodium cyanide and copper cyanide; molten copper has also been treated with sodium cyanide followed by a 30% alloy of calcium and copper 90 as a degasifier. Other degasifiers can be used to eliminate blow-holes which might be caused by occluded gases.

In the treatment of steel with sodium cyanide, the procedure was in general to drop broken pieces of sodium cyanide, preferably contained 95 in paper envelopes, into the ladle and then immediately pour the molten steel from a large ladle over this cyanide. There was no violent spattering reaction, but on contact of the molten metal with the cyanide, dense white fumes are developed which subside in a short time; this is followed by an evolution of gases from the metal. The metal is held until the evolution of gases from the molten metal has ceased, whereupon the metal is cast.

The treatment of copper with cyanide materials has been carried out in several ways. In the first place, molten copper has been poured over sodium cyanide. Secondly, it has been poured over copper cyanide; and finally, the 110

cyanide materials have been added to the molten copper. Either of the methods is satisfactory. For example, three ounces of 96-98% sodium cyanide lumps were added to 150 lbs. of molten copper. The cyanide was first placed in a graphite phosphorizer which had small holes bored through the top of the cup to assist in assuring contact of molten sodium cyanide with the copper melt. Sodium cyanide was added just before pouring the metal and sufficient time allowed for the generated gases to boil out. The flux, consisting of lime and sodium-borate as a slag, was left on the copper during the treatment with sodium cyanide. Copper has been treated when melted in a reducing atmosphere, keeping the crucible covered; and also in an oxidizing atmosphere. No difficulty was experienced with the introduction of the sodium cyanide into the copper. The castings obtained showed conductivities much better than the conductivity of the untreated copper.

Further, copper which has thus been treated with sodium cyanide, was degasified by means of a 30% alloy of calcium and copper; this resulted in castings having a very high conductivity.

I claim:

1. Method of improving the properties of copper or its alloys which comprises treating said copper or alloys thereof in the molten state with copper cyanide.

2. Method of improving the properties of copper or its alloys which comprises treating said copper or alloys thereof in the molten state with copper cyanide and thereafter degasifying the melt.

3. Method of improving the properties of copper or its alloys which comprises treating said copper or alloys thereof in the molten state with copper cyanide and thereafter degasifying the melt with a copper-calcium alloy.

80

35

90

95

WILLIAM F. ZIMMERLI.

25

100

30

105

35

110

40

115

45

120

50

125

55

130

60

135

65

140

70

145

75

150